

April 18, 1961

H. SEGHEZZI

2,979,928

HIGH-STRETCH KNITTED FABRIC

Filed Sept. 6, 1957

*Fig.1*



*Fig.2*



*Fig.3*



*Fig.4*



INVENTOR.  
HANS SEGHEZZI  
BY *Richards & Geier*  
ATTORNEYS

1

2,979,928

## HIGH-STRETCH KNITTED FABRIC

Hans Seghezzi, Linsenhofen, Kreis Nurtingen, Germany

Filed Sept. 6, 1957, Ser. No. 682,378

5 Claims. (Cl. 66—196)

This invention is concerned with improvements in or relating to high-stretch knitted fabric.

Fabrics having high-stretch are normally produced by one of two processes. In one process, rubber threads are worked into the material or the material is treated with a rubber solution; in the other method, the fabric is made from crimped polyamide yarn.

Material produced by either of these processes has a number of serious disadvantages.

In using rubber one has to take into account its unfavourable wearing properties. Thus, rubber is unpleasant to wear next to the skin, is frequently insufficiently permeable to air and has an unpleasant smell. Moreover, it does not age well, for it becomes brittle on prolonged use in the atmosphere, especially in the presence of skin oils. Furthermore a material having rubber threads can hardly be repaired when damaged, since one cannot tie together exposed and broken rubber threads.

Knitted fabric made from crimped polyamide threads can become unpleasant looking owing to the drawing of capillary fibres, and moreover crimped polyamide yarn is sensitive to the action of sunlight. When greatly stretched, knitted fabric made from polyamide yarn can become transparent.

In view of this, it is clear that the hitherto known high-stretch yarns and knitted fabrics have important disadvantages in respect to wearing and ageing properties.

It is the object of the present invention to provide an improved high-stretch knitted fabric.

The knitted fabric according to the invention is particularly suitable for the production of swimming suits, bandages, welts, and the like close-fitting material, it can be stretched both lengthwise and breadthwise, and does not become transparent even when greatly stretched; it is pleasant to wear on the skin, it has high resistance to ageing under the action of the atmosphere, light, grease and oil. It does not readily produce drawn fibres. Any damage to individual loops of the knitted material can be repaired in a simple manner.

Moreover, synthetic yarns can be used for the production of the knitted fabric according to the invention in such a manner that their favourable properties are brought into prominence without their known disadvantages having much substantial effect on the practical value of the knitted fabric.

This object is achieved in the knitted fabric according to the invention by the use of two different yarns and by the special manner of their arrangement.

According to the invention there is provided a high-stretched knitted material comprising a double-sided knit from a bulky yarn and a one-sided knit from a fine, more stretchable yarn, the two knits being worked into each other so that the one-sided knit forms an intermediate layer between the two sides of the double-sided rib knit both in unstretched or stretched conditions.

The bulky yarn in addition to having a high volume, preferably has good wearability, high resistance to ageing

2

in the atmosphere and light, and as high as possible an absorption coefficient for UV-radiation. Its elasticity can be low. Preferred yarns for this purpose are polyacrylonitrile worsted yarns.

5 The fine yarn should be as elastic as possible and should retain its stretch even over long periods of stretching. On the otherhand it need not be immune to the effect of sunlight and mechanical rubbing and can even have bad wearing properties. The known crimped yarns of high stretch can therefore be used for this purpose. Preferably, set crimped polyamide yarns are used.

The arrangement of these two yarns is very important. A rib knit from the bulky yarn and a single sided knit from the fine yarn are so worked into each other that the loops of the single-sided knit come to lie neither on the upper- nor on the underside of the rib knit, but form an intermediate layer between the two sides. The rib knit has a relatively large length of thread between the two loop surfaces. Owing to its high stretch, 20 the fine yarn draws its own loop heads beneath the level of the knit from the bulky yarn, and at the same time draws the entire knitted fabric together so strongly that the loops of the knit which is ribbed and double-sided lie very close to one another on the surfaces. As a 25 result, the knitted fabric has a pleasant appearance.

On stretching the knitted fabric according to the invention the threads of the knit from the fine yarn are tensionally stressed, whereas the knit from the bulky yarn, owing to the large length of thread between the 30 two loop surfaces, can follow the stretching without substantial stress. The limit of stretch of the knitted fabric is hence determined by the rib knit. Upon reaching the limit of stretch, the fine yarn does not become fully extended and hence still is nontransparent.

35 The accompanying drawings show in section a preferred embodiment of knitted fabric according to the invention.

Figure 1 is a plan view showing a ribbed knit from a bulky yarn; the great length of thread between the two 40 loop surfaces will be observed.

Figure 2 shows a single-sided plain knit from fine crimped yarn. The knit is very flat in comparison with that of the previous figure.

Figure 3 illustrates the manner in which the two knits 45 are worked into each other according to the invention. The knitted fabric is shown in unstretched condition.

Figure 4 shows the same knitted fabric stretched nearly to the elastic limit.

Figures 3 and 4 make it clear that the upperside and 50 the under-side of the knitted fabric are formed exclusively of loops of yarn 1, whereas the flat unit from yarn 2 does not appear on the surface.

It is apparent that the arrangement of the knitted fabric can be modified in various ways without interfering 55 with the basic arrangement of the knitted fabric according to the invention. Thus, for example, additional relief ribs and relief patterns can be knitted in.

In order that the invention may be well understood, it will now be described with reference to the following 60 example which is given by way of illustration only.

As yarn 1 there is used polyacrylonitrile worsted yarn whereas set, crimped polyamide thread which can be stretched by about 500% is used as yarn 2. By the use of these synthetic materials the resultant knitted fabric 65 is mothproof, remains felt-free, and hence airpermeable, and dries quickly.

The knitting is carried out on an interlock circular knitting machine which must have two needle carriers, the one carrier having twice the number of needles as the 70 second carrier, and the needles of the second carrier being exactly in line opposite some of the needles of the first carrier. The machine operates in such a way

that the opposed needles cannot be projected at one feed at the same time, but so that one feed projects some of the needles of the two carriers at the same time, and another feed projects the needles of the first carrier only.

The rib web must allow the fabric a high expansion without substantial stress of the rib web thread, since the exertion of high elasticity power is the object of the plain web, and it further must allow the stitches of the plain web to withdraw within the fabric.

The bulky yarn 1 for the ribbed web is delivered to the first feed as it is done on ordinary rib knitting machines, the finer yarn for the plain web is, fully stretched, fed to second feed and forms plain knit stitches on the needles in succession.

Furthermore, since the consumption of yarn 2 compared with yarn 1 is reduced owing to the flat plain web and the small loops, and in order to provide for a faultless formation of the stitches, the quantity of thread for the plain web must be regulated through some type of lock or, better, a thread regulator the drive gear of which has about 40% less teeth than that of the thread regulator for the ribbed web.

The rib knit thus produced has good resistance to direct exposure to sunlight, a pleasant hand, high heat-retaining capacity, rapid drying properties, and substantially constant stretch even in wet condition. The high stretch of the single-sided knit from polyamide yarn enables the fabric to contract very strongly. Both knits have high resistance to oil and alkalis.

Although the described embodiment shows many advantages, the invention is in no way restricted to the use of interlock-circular knitting machines. Thus, for ex-

ample, one may use a flat knitting machine provided with an interlock needle position, and if desired, thread regulators need not be used.

The claims defining the invention are as follows:

- 5 1. A high stretch composite knitted fabric, comprising a rib fabric consisting of a bulky yarn and a fabric consisting of a fine highly stretchable yarn, the two fabrics being interknit so that the second-mentioned fabric forms an intermediate layer between the two sides of the first-mentioned fabric.
- 10 2. A composite knitted fabric according to claim 1, wherein the first-mentioned fabric has the same appearance on both sides and wherein the second-mentioned fabric is plain knitted and forms the intermediate layer both in unstretched and stretched conditions of the composite fabric.
- 15 3. A composite knitted fabric according to claim 1, wherein the first-mentioned fabric consists of a bulky polyacrylonitrile worsted yarn.
- 20 4. A composite knitted fabric according to claim 1, wherein the second-mentioned fabric consists of a set, crimped polyamide yarn.
- 25 5. A composite knitted fabric according to claim 1, said composite fabric having additional knitted-in ribs.

#### References Cited in the file of this patent

#### UNITED STATES PATENTS

|           |               |               |
|-----------|---------------|---------------|
| 1,087,690 | Scott et al.  | Feb. 17, 1914 |
| 2,009,361 | Lawson        | July 23, 1935 |
| 2,503,444 | Lawson et al. | Apr. 11, 1950 |
| 2,755,616 | Weller        | July 24, 1956 |